

Jan. 24, 1939.

C. BIRDSEYE ET AL

2,144,673

INCANDESCENT LAMP AND ITS MANUFACTURE

Filed Oct. 31, 1935

Fig. 1.



Fig. 2.



Fig. 3.



Fig. 4.



Fig. 5.



Fig. 6.



Fig. 7.



Fig. 8.



Fig. 9.



Fig. 10.



Inventors

Clarence Birdseye and  
Pinus Doren.

by Kenway & Witter  
Attorneys

## UNITED STATES PATENT OFFICE

2,144,673

INCANDESCENT LAMP AND ITS  
MANUFACTUREClarence Birdseye and Pincus Deren, Gloucester,  
Mass., assignors to Birdseye Electric Company,  
Gloucester, Mass., a corporation of Delaware

Application October 31, 1935, Serial No. 47,581

11 Claims. (Cl. 176—34)

This invention relates to the manufacture of incandescent lamps and more particularly to such lamps in which the bulb is provided with a reflecting surface for increasing the amount of light from such a source available for useful work.

In the manufacture of incandescent lamps of the kind having a reflecting lamp bulb certain of the light rays from the bright filament of the lamp are intensified by reflection from a reflecting surface formed by silvering a part of the wall of the bulb. For direct lighting the filament is hooded by the reflector, the lower limit of the silvered area being preferably at such a distance from the filament that all of the rays emanating from the filament, both direct and reflected, eventually will leave the lamp within a predetermined field. Practice has indicated that the maximum useful luminous field of such a lamp may be approximately defined by the base of a 60° cone. Accordingly, in general, the chosen relation of the depth or boundary of the reflecting surface relative to the filament for direct lighting is such that the path of the outer light rays passing outward from beneath said reflecting surface is approximately 60° to the vertical. For indirect lighting the reflecting area may be above, below or at one side of the filament according to the position of the lamp when in use and the above described relation of the boundary of the reflector to the filament may be varied considerably for indirect lighting, where the area of the illuminated field may profitably be very greatly increased. It has been found that in either case the efficiency of the lamp is increased by the use of a reflecting bulb and in the case of direct lighting there is the further advantage of having the intensely bright spot of the filament effectively removed from the field of vision.

In developing a commercially successful reflecting bulb for incandescent lamps several difficulties were encountered and largely overcome but in the solution other disadvantages developed which this invention has eliminated.

One part of the problem was to eliminate from the useful field of light any projected image of the filament. Such a projection of a distorted image of the filament, thereby making a very bright area in the illuminated zone is due to the fact that the filament is preferably located at or near what may be described as the "focus" of the reflecting surface of the bulb. Heretofore, the solution of this problem has been attempted by frosting the lower or useful light emitting area of the bulb below the silvered or reflecting area, or above it, in the case of lamps having the lower portion of the bowl silvered. This treatment will diffuse the useful light to a certain extent and so tend to eliminate the discordant bright area, but

with considerable increased loss of light, as explained below.

Another part of the problem was to eliminate any tendency of the lamp to cast a shadow of the filament near the center of the brightly illuminated field due to the reflected light impinging in part on the filament itself. This shadow tends to center with the reflected image of the bright filament, but because of the irregularity and non-symmetry of the parts of the filament and because they are not located at any true focus of the reflecting area, the shadow and the bright image do not register but there is built up a zone that is of different brilliancy than the rest of the illuminated area, most of which is brighter but with a mottling of shadow. A diffusion of the emitted light by frosting as above described has heretofore been resorted to in an attempt to solve this problem, and with similar introduction of losses.

Frosting the area of the bulb through which light is emitted has a serious disadvantage in that the high concentration of the bright rays passing through the frosted glass tends to unduly raise the temperature of the glass due to the absorptive power of the frosting, and this increased loss as heat represents a substantial loss of useful light.

One object of the present invention is to increase the efficiency of reflecting lamps by eliminating high-lights and shadows within the useful lighting zone all without decrease in intensity of either the direct or reflected light rays from the source of light.

In achieving this object a new method is employed of producing a diffused light from a high-temperature source of light which is particularly useful in connection with a reflecting bulb incandescent lamp. Such new method is characterized by a diffusion in a heterogeneous manner of reflected light rays from the source of light, for example from the filament of an incandescent lamp, thus neutralizing any distinct focusing effect and producing a substantially uniform intensity of illumination throughout the lighted area without loss of efficiency. The employment of this new method permits the manufacture of reflecting bulb incandescent lamps with clear glass below the reflecting area thus allowing all of the light rays, in undiminished brilliancy, to illuminate the useful field.

This invention, in its broader aspects, embraces within its field the diffusion of light through the medium of a diffusing reflector in contradistinction to the diffusion of light by transmitting through a diffusing body. A particular application relates to diffusing the light from reflecting bulbs so as to eliminate from the illuminated field either the partially focused image or the shadow of the filament or other source of light.

In order that the later use of the term "diffus-

ing reflector" may be understood the distinction between reflected light with and without diffusion should be borne in mind. In an ordinary or plane reflector having a smooth reflecting surface or 5 mirror the angle of incidence is always equal to the angle of reflection from the particular point under consideration. When the reflecting surface is not a single plane, for example a curved surface, these angles are measured with respect 10 to a plane tangent to the surface at the point in question. Thus at any point on such a curved reflecting surface the light rays are still directly reflected and at all points the two angles are always equal. Such smooth reflectors provide 15 specular reflection.

In a diffusing or non-specular reflector the angle of reflection at any point on the surface may be any angle whatever with respect to the general contour or surface plane of the reflector. 20 That is, although by chance certain rays and beams may be reflected at the angle of incidence, practically all of the rays and beams falling on a diffusing reflector will be reflected at an angle different from the angle of incidence with respect 25 to the surface plane of the reflector. A diffusing reflector will therefore have a very large number of minute or microscopic surface irregularities which individually may form almost any angle whatever with the plane of the reflector as a 30 whole. Each of these microscopic surface irregularities acts as an individual mirror and the angles of incidence with respect to the surface plane of the reflector and reflection from each individual mirror are, of course, equal. Reflected light 35 from such a mirror is diffused, that is it leaves the mirror in almost all possible directions.

A specific application of the invention in commerce is to incandescent lamp bulbs having a portion of the wall of the bulb prepared as a 40 highly efficient diffusing reflector. The lamp bulb may be of the conventional shape or of almost any special shape and yet gain a pronounced beneficial effect by having some part of its surface acting as a diffusing reflector. In any 45 application of the invention to lamp bulbs the surface of that part of the wall of the bulb acting as the reflector may have been modified either at the time of making the bulb or by a subsequent treatment enabling diffusion of light, or modified 50 by the kind of reflecting surface applied to create a diffusing reflector, its roughened, irregular or uneven reflecting surface being formed either before or after or during the operation that produces the reflector itself.

55 In the past, difficulties have been encountered in producing an efficient, durable and attractive reflecting silver film on the inner surface of an evacuated glass vessel or one to be evacuated. These difficulties are no doubt responsible for the 60 fact that prior to my work no satisfactory inside-silvered lamp bulb was commercially available. One difficulty was that it was found impossible to make a silver film adhere evenly and uniformly to the inside surface after evacuation. The silver 65 could be deposited by any well-known process, but when the bulb was thereafter evacuated, bubbles would make their appearance in the silver film which, on bursting, would permit the silver to peel off the glass wall.

70 It was subsequently discovered that the difficulty was due to a physical and possibly chemical change of the surface layer of the glass, after which change the layer readily occluded gases because of its more spongy nature. The usual 75 cleaning processes employed in the art produced

little or no effect on this layer, so that upon evacuating the bulb, the occluded gases would expand and give rise to the bubbles which destroyed the continuity of the silver film.

In copending application, Serial No. 42,227, filed September 26, 1935, Pincus Deren describes the mentioned difficulties and discloses a method of eliminating this injurious gassy layer without affecting the transparency of the bulb, by a variation of the well-known etching process. It is also a part of our invention to eliminate the gassy layer prior to silvering, but, since my primary interest is in a diffusing surface and my preferred means for obtaining it is to etch or frost the inner surface of the bulb prior to silvering, we may use any common etching or frosting solution, preferably one giving a good even and uniform frost with no marked depressions. When, on the other hand, we desire to deposit silver on a smooth transparent surface, we may utilize the etching solution disclosed by Deren for this purpose. In either case, the etching process serves to remove the objectionable gassy layer and prepare the inner surface of the bulb for receiving the deposited silver in such a way that after 25 silvering and evacuation, a fine, attractive silver film is obtained having no holes, bubbles or peeled spots. By depositing the silver upon a roughened or frosted glass surface we have found that the film adheres very strongly. 30

A further problem arises in the case of inside frosted bulbs by reason of the fact that the inside frosting process seriously weakens the glass, presumably by the formation of myriads of minute crevices at the bottom of which the thickness of the glass is below the safe limit. In the past it has been necessary to give to inside frosted bulbs a second etching and strengthening treatment which necessarily adds to the cost of production. Such a strengthening treatment, now 40 widely employed in the manufacture of inside-frosted non-reflecting bulbs, is disclosed in U. S. Letters Patent No. 1,687,510, to Pipkin.

We have found that such second strengthening treatment is wholly unnecessary in the case of 45 my inside frosted, silvered bulbs, because the silver film coats the sharp crevices and strengthens the surface. Our inside frosted silvered bulb, though given no other strengthening treatment, is adequately strong for shipment and commercial use in general. 50

The objects of the invention and the features and methods through which they are attained will best be understood and appreciated from the following description of the best embodiments at 55 present known as illustrated in the accompanying drawing.

The figures of the drawing are sectioned for glass as the base material for the reflector but this is for illustration in connection with a use of 60 the invention in incandescent lamps and is not to be construed as limiting. In the drawing:

Figures 1 and 2 show, respectively, a pre-treatment of the base material by frosting and a reflecting medium is then applied to such frosted 65 face, as by silvering;

Figs. 3 and 4 show, respectively, one face of the base material prepared for retaining an irregular surfacing of the reflecting medium and such surfacing then applied; 70

Figs. 5 and 6 show, respectively, a modification of the treatment shown by Figs. 3 and 4 in that the prepared base material is given its uneven reflecting surface by a special treatment thereof;

Figs. 7 and 8 show, respectively, a modification 75

of the treatment shown in Figs. 1 and 2 in that the base material is first molded to an uneven matrix prior to applying a reflecting medium to a face thereof;

5 Fig. 9 is illustrative of an incandescent lamp provided with a diffusing reflector made in accordance with the teaching of this specification; and

10 Fig. 10 is a view of an incandescent lamp similar to Fig. 9 but showing a modified form of reflector for reflecting both diffused and non-diffused light.

15 Referring to the drawing, 10 represents a section of a suitable base material for a reflector or for a mirror which may be a part of the glass bulb of an incandescent lamp. The four pairs of figures from 1 to 8 illustrate four methods of procedure to produce a diffusing reflector on the base material. These will be described in their 20 application to the production of reflecting lamp bulbs as a specific example of use within the broader scope of the invention.

Method I (Figs. 1 and 2)

25 The interior of the bulb may be frosted by a pre-treatment with hydrofluoric acid in the manner regularly employed in the industry for ordinary non-reflecting bulbs except that a single etching process is sufficient as above described. 30 The frosted area may be the entire inside surface of the bulb, or it may be co-extensive with the reflecting surface, or it may be of less extent than the reflecting surface which will be obtained by silvering at a later operation. It is preferable, from the standpoint of efficiency, to 35 leave the light transmitting area of the bulb unfrosted but for certain purposes it may be desirable to frost the light transmitting part of the bulb beyond the diffusing reflector, so that the bright filament will not be directly visible 40 from any angle. A thin coating of metallic silver deposited on the microscopically roughened surface forms a rougher matte surface than when deposited on the smooth glass; in fact it partakes almost exactly of the nature and contour of the 45 minute craters and pin holes which have been etched into the surface of the glass by the hydrofluoric acid. While the surface appears to be macroscopically smooth the rugosities thus formed are readily visible under the microscope. 50 This minutely irregular surface of metallic silver is still silver and it still reflects with the high coefficient of reflection that any silvered surface does, but it reflects a diffused light.

55 The coating resulting from this method of solving the problem gives a white appearance to the outside of the bulb, even whiter than an unsilvered frosted bulb. For certain purposes this may well be an advantage in that the bright diffusing reflector is not visible through the glass.

60 Under some conditions, as in the case of an asymmetric bulb designed for a special purpose, it may not be desirable or necessary to form a light diffusing surface over the entire area of its reflector. In such a case the reflector would consist of a combination of selected areas for reflecting a diffused and a non-diffused light.

An alternative method involves frosting either the inside or the outside and silvering the outside of the bulb. This will also produce a diffused reflected light, but because it has several disadvantages it is not the preferred method. There is always the danger of the unprotected silver becoming defaced, as by scratching, during the period of use, and it will tarnish and eventually

deteriorate. A protector against these eventualities may be provided but this is expensive and for many uses undesirable. Moreover the light, in order to be reflected from the silvered outside surface of the bulb, must first pass through the glass and in the case of inside frosting must pass through the glass twice. This causes a real loss of lighting efficiency.

Method II (Fig. 3 and 4)

10 This method involves the deposition of a relatively coarse coating of silver on the inside of an unfrosted bulb. This can be accomplished by first applying a thin relatively smooth coating of silver, while maintaining the bulb and its contents of 15 the silver depositing solution in active motion as disclosed in the mentioned Deren application, and then at the end of the period when an adequate deposit of the fine crystals has taken place, the shaking motion imparted to the bulb and its contents is stopped, and the continued deposition of 20 silver is allowed to proceed while the bulb is at rest. This builds up a relatively thick and irregular deposit upon the first coating which appears under the microscope to be composed of large 25 crystals, and crystal masses. These large relatively irregular crystals have the same excellent high coefficient of reflection as any other pure silver coating, but are actually sufficiently large and irregular to reflect a diffused light. It has 30 been found that this relatively coarse crystal deposit adheres better to the glass if it is deposited upon a finer coating of silver, but this method is not limited to this combination of layers since satisfactory diffusing reflectors may be made by 35 a coating of coarse silver crystals directly onto the base material.

Method III (Figs. 5 and 6)

40 This method consists in depositing a regular fine coating of metallic silver, as described in said co-pending application Serial No. 42,227 of Pincus Deren, and then making this relatively smooth surface somewhat coarser and rougher by attacking it with a chemical substance that will change 45 part of the silver to a compound of silver. Since the very fine crystals of which the metallic silver layer is composed fit very closely together, and may even overlap in places, it is apparent that by changing some of these crystals and/or parts of some of these crystals to a compound containing 50 a greater weight of matter and of lower specific gravity than the heavy metallic silver, the volume of the silver coating will be considerably increased. This effect will be manifest by an irregular raising of parts of the surface of the deposit and the development of what appear to be 55 larger crystals. The color of the deposit may change somewhat, depending on what the treatment is. For example, if the freshly silvered bulb is filled with a solution of sodium chloride there will be a gradual change of the surface layers of the silver coating from silver to silver chloride. Red phosphorous in water suspension introduced 60 into the bulb will gradually attack the surface of the silver deposit, particularly if a trace of non-oxidizing mineral acid, for example hydrochloric, is added to the water. Air containing a very low concentration of chlorine, or other halogen, may be admitted into the dry bulb and again part of 65 the silver deposit is changed to silver chloride.

Method IV (Figs. 7 and 8)

70 This method of forming a highly efficient reflector producing diffused light may be carried out 75

by using special molds or matrices in which the bulbs are blown. Any repeated pattern or a series of geometric lines may be cut into or raised upon the bulb mold, such as a pattern made by forcing a light screen into molding clay, and located so that the part of the bulb subsequently to be silvered or otherwise made into a diffusing reflector surface will have this pattern upon the base material. Thus, while the pattern will be blown into the outside of the bulb this same pattern will be carried through to the inside of the bulb and will form an uneven inner surface. This inside surface, the roughening of which should simulate as closely as possible the minuteness of the rugosities of frosting, can then have a thin smooth coat of metallic silver applied thereto and as this provides a roughened or uneven reflecting surface a diffusing reflector will result.

A diffusing reflector made under any of these methods greatly increases the amount of diffused light emanating from such a reflecting surface occupying a definite and predetermined part of the surface of the bulb of an incandescent lamp, and so avoids either the projection of a partially focused image of the filament or its shadow, and without necessarily causing the light to be transmitted through a frosted or otherwise diffusing surface with its consequent loss of efficiency.

This difference in lighting efficiency is shown by the following laboratory data, typical of many such comparisons that have been made. The bulbs of the two lamps compared were as nearly alike as possible in all respects, except that the bulb of lamp B was frosted over the light-transmitting, non-silvered area only, and the bulb of lamp A was frosted under the silvered area only. Both were 150 watt reflecting and diffusing lamps, but lamp A obtained diffusion by reflecting from a diffusing inside reflector with a microscopically roughened surface the light being transmitted through unfrosted glass, while lamp B reflected from a bright plain inside reflector and obtained diffusion by transmitting the light through frosted glass. The light falling on the test table was substantially equally diffused and both luminous fields were substantially uniform as to intensity of illumination.

The lamps were tested in the same socket, permanently fastened at a constant distance above the test table. The actual foot-candles of illumination falling on the table were measured directly under the lamp and at one half foot distances measured in a straight line along the table away from this point.

| Distance from point directly under lamp in feet | Lamp A diffusing-reflector type, foot-candles | Lamp B frosted over transmitting area, foot-candles |
|-------------------------------------------------|-----------------------------------------------|-----------------------------------------------------|
| 0.0                                             | 48.0                                          | 41.0                                                |
| 0.5                                             | 50.0                                          | 42.0                                                |
| 1.0                                             | 42.5                                          | 41.0                                                |
| 1.5                                             | 37.5                                          | 37.5                                                |
| 2.0                                             | 33.0                                          | 31.5                                                |
| 2.5                                             | 27.5                                          | 26.0                                                |
| 3.0                                             | 23.5                                          | 22.0                                                |
| 3.5                                             | 20.0                                          | 18.0                                                |
| 4.0                                             | 18.0                                          | 14.0                                                |
| 4.5                                             | 14.5                                          | 12.0                                                |
| 5.0                                             | 11.5                                          | 10.0                                                |
| 5.5                                             | 9.5                                           | 8.0                                                 |
| Totals                                          | 335.5                                         | 303.0                                               |
| Volts                                           | 120                                           | 120                                                 |
| Amperes                                         | 1.265                                         | 1.275                                               |
| Watts                                           | 151.8                                         | 153.0                                               |

Thus, in this comparison, despite the fact that the prior art lamp B, obtaining diffusion by transmitting through a frosted area, was of slightly

higher wattage rating, it actually emitted less light. The sum of the foot-candles in each of the columns is a rough comparative measure of the total amount of light emitted. On comparing these sums it is apparent that the new diffusing-reflector lamp A of this invention emits about 10% more light than the old reflecting and diffusing lamp B.

While silver has been named as a metal suitable for a reflecting coating it is contemplated that other metals may be employed within the scope of the invention. For example, nickel may be used, or chromium may be deposited upon a thin priming coat of silver.

Fig. 9 of the drawing shows an application of the invention to an incandescent lamp used for direct lighting. As illustrated the diffusing reflector 12 is of sufficient depth to hood the filament 14 the lower boundary of the reflector being so located relatively to the filament that the light rays may spread to an approximate 60° cone, indicated by dotted lines, hereinbefore described as having been found to constitute an efficient field of useful light. With the use of a diffusing reflector the portion 16 of the bulb wall through which the light shines may be clear glass as shown. The figure shows a reflecting disk 18, preferably of metal, and located between the filament and seal of the lamp serving, among other functions, to reinforce the useful light emitted by deflecting the rays or beams heretofore lost in the neck of the lamp, as disclosed in the pending application of Clarence Birdseye Serial No. 33,694, filed July 29, 1935 which is Patent 2,142,104. This reflecting disk, when used with the diffusing reflector 12, would also preferably be converted to a diffusing reflector by one of the methods described herein or its equivalent.

Fig. 10 illustrates, by way of example, an incandescent lamp provided with a reflector that reflects a diffused light from one part and a non-diffused light from another part. The bulb shown is provided with an inside diffusing reflector 12 like that shown in Fig. 9 and with an added plain or specular reflector 20 in the form of an annulus 45 at the lower edge of the reflector 12. The position of the specularly reflecting portion with relation to the diffusing portion may be varied. It may be added to or it may partly impinge upon or be wholly surrounded by the diffusing reflector according to the conditions under which the lamp is to be used, for example, spot lighting a particular object or increasing the illumination over a special area.

When the specularly reflecting portion is in the position shown in Fig. 10, namely, an annulus at or about the region of greatest diameter of the bulb, it serves to increase the illumination over a ring at the periphery of the illuminated field where it would otherwise be less than at the center. At the same time it also serves to narrow the field somewhat. The net effect is to give a more uniform illumination over a narrower field instead of a less uniform illumination over a wider field. When the specularly reflecting portion is otherwise disposed it gives a different effect, predictable from its position relative to the filament.

From the foregoing description and from the appended claims it will be understood that diffusing reflectors to be manufactured from the teaching of this invention are not limited as to size, shape or location with respect to the source of light and may be employed with lamps varying widely in type and power. In its application

to what are known to the trade as "incandescent lamps", the invention is inclusive of all such lamps capable of diffusing light without causing it to be transmitted through a diffusing medium, or capable of diffusing light simultaneously with its reflection from a reflecting surface, particularly an internal reflector and light diffuser.

5 It is believed that a reflector of this type, having a surface of high reflective index and with this surface minutely roughened in a manner 10 readily discernible under a microscope, and for the purpose of reflecting a diffused light from a high temperature concentrated source, and without transmitting this reflected light through a diffusing medium which always incurs losses, has 15 not been heretofore available.

10 The nature and scope of the invention having been indicated and preferred embodiments and methods of manufacture having been specifically 20 described, what is claimed as new, is:—

1. The method of making light diffusing lamps having a high temperature source of light which comprises applying a substantially smooth coating of silver to a surface of the lamp and then 25 treating the exposed surface of said coating in a manner to create surface rugosities.

2. The method of claim 1 in which the said treatment consists in superimposing an irregular deposit of relatively large silver crystals and silver 30 crystal masses on said first coating of silver.

3. The method of claim 1 in which the said treatment consists in attacking the outer layers of said coating with a chemical capable of converting the treated parts to a compound of silver 35 thereby obtaining an uneven development of larger crystals throughout the treated parts and thus raising such parts irregularly above the surface of said coating.

4. The method of claim 1 in which the said 40 treatment consists in increasing the volume of the silver in said coating throughout parts of its surface thereby raising said parts above the surface of said coating.

5. The method of making light diffusion lamps 45 having a high temperature source of light which comprises coating a surface of the lamp with a deposit of silver crystals sufficiently large and irregular to produce a surface capable of reflecting a diffused light.

50 6. An incandescent lamp including in its struc-

ture a bulb and a light source and having a metallic reflecting medium applied to the inner surface of part of the area of the bulb, the reflecting medium having its exposed surface uneven so that light reflected thereby is diffused, said inner surface of the bulb to which the reflecting medium is applied being smooth and even and the exposed surface of the reflecting medium being rough and uneven.

7. An incandescent lamp having a reflecting 10 disc positioned between the source of light and the seal of said lamp, said disc having its reflecting surface roughened by minute irregularities so that it reflects a diffused light.

8. An incandescent lamp having a reflecting 15 disc positioned between the source of light and the seal of said lamp and having a reflecting medium applied to a predetermined area of its bulb, the reflecting surfaces of both disc and bulb reflecting a diffused light by virtue of minute 20 irregularities extending thereover.

9. An incandescent lamp comprising a bulb having a filament of concentrated spiral form therein, the inner surface of said bulb being provided with a reflecting surface from a point on 25 the neck of said bulb to the region of greatest diameter of said bulb, an annular portion of said reflecting surface in the region of greatest diameter of said bulb being specularly reflecting in character and the remainder of said reflecting 30 surface being diffusely reflecting in character, the filament being placed substantially at the focus of said diffusely reflecting portion of said reflecting surface, and the plane angle subtended at the filament by that boundary of the specularly reflecting surface which is furthest from the 35 neck of said bulb being substantially 120 degrees.

10. An incandescent lamp as in claim 9 in which the diffusely reflecting surface consists of a film of metal of substantially uniform thickness 40 adhering closely to the roughened inner wall of the bulb.

11. An incandescent lamp as in claim 9 in which the diffusely reflecting surface consists of a film of metal adhering to the smooth inner 45 wall of the bulb, the exposed surface of said film being rough.

CLARENCE BIRDSYE.  
PINCUS DEREN.